

Patented June 5, 1928.

1,672,803

## UNITED STATES PATENT OFFICE.

HELENE CHONLA, OF EL PASO, TEXAS.

### HANDKERCHIEF.

No Drawing.

Application filed December 4, 1926. Serial No. 152,721.

The present invention relates to improvements in handkerchiefs and method of making same, and has for an object to provide a handkerchief of tissue paper, treated to eliminate rustle and stiffness from the paper, to render same soft and pliable and avoid rumpling.

The invention also aims to provide a handkerchief, which will be cheap and sanitary, and which will dispense with laundering.

With the foregoing and other objects in view, the invention will be more particularly described hereinafter and pointed out in the subjoined claims.

15 The improved handkerchief is formed in any suitable size from tissue paper or other appropriate material. This material is initially treated by floating it hastily through a preparation of ten parts of ammonia to two parts of glycerine. The ammonia employed is preferably eight parts 20 aromatic spirits of ammonia and two parts crude undiluted ammonia. The paper is thereafter dried in flat sheets and is subsequently drawn quickly through a preparation 25 of three parts of peroxide of hydrogen, commonly referred to as "peroxide" to one part of glycerine. Again, the material is carefully dried in straight flat sheets, and 30 is then ready for cutting and use.

The ammonia toughens the paper, gives it body and partially softens the same through the addition of the glycerine.

The ammonia also fortifies the paper 35 against the dissolving effect of the peroxide. The peroxide, however, is the only medium so far discovered, which will entirely aid the glycerine to soften the paper and eliminate

the resulting noise. The peroxide also counteracts the unpleasant oily effect of the 40 glycerine on the paper.

After use, the handkerchief so made and treated may be easily disposed of by fire or water.

I have described a preferred and satisfactory construction of handkerchief and preferred steps of a method for treating same, but I desire to be understood that various changes may be made in such construction and steps, without departing from 50 the spirit of my invention, provided same come within the scope of the following claims.

Having thus described my invention, what I claim and desire to secure by Letters 55 Patent of the United States is:

1. An improved handkerchief of paper treated with ammonia, glycerine and peroxide.

2. A method of treating paper handkerchiefs, which consists in initially treating the paper with a preparation of ammonia and glycerine, subsequently drying the material, then treating same with a preparation of peroxide and glycerine and again drying 65 the paper.

3. The herein described method of forming tissue paper handkerchiefs, which consists in initially treating the paper with a preparation of 10 parts ammonia and 2 parts 70 glycerine, then drying the material in flat sheets, subsequently drawing the flat sheets through a preparation of 3 parts of peroxide to 1 part of glycerine, and again drying the material in flat sheets.

HELENE CHONLA.